

# UNITED STATES PATENT OFFICE.

FRANK A. WILMOT, OF BRIDGEPORT, CONNECTICUT.

## MANUFACTURE OF IRON AND STEEL.

1,012,810.

Specification of Letters Patent.

Patented Dec. 19, 1911.

No Drawing.

Application filed January 27, 1911. Serial No. 605,015.

To all whom it may concern:

Be it known that I, FRANK A. WILMOT, a resident of Bridgeport, in the county of Fairfield and State of Connecticut, have 5 invented a new and useful Improvement in the Manufacture of Iron and Steel, of which the following is a full, clear, and exact description.

My invention relates to the manufacture 10 of steel and is designed to provide an improved method by which steel may be more cheaply and rapidly produced than heretofore.

The invention generally stated, consists 15 in smelting iron ore in a blast furnace without regard to analysis as regards silicon in the pig produced, and preferably also as to sulfur and phosphorus, giving a product relatively high in silicon and preferably 20 also in phosphorus and sulfur. That is, there is no proportioning the charge so as to bring the content of these metalloids within the proportions required for basic or Bessemer pig. The molten pig metal 25 from a blast furnace or furnaces operated in this manner is taken to a large regenerative tilting furnace of the open hearth type in which a constant pool is maintained. In this mixer, the metal is given a preliminary 30 open hearth treatment, but at a low temperature compared with that of ordinary open hearth methods. For example, the temperature may be 1000° F. lower than the ordinary temperature of open 35 hearth manufacture, as in the primary furnace described in the United States patent to W. R. Palmer, No. 924925, granted June 15th, 1909. From this mixer, charges are 40 taken to make a portion or the whole of a charge for an open hearth furnace of the ordinary type.

In carrying out my invention, I employ 45 one or more blast furnaces, a regenerative tilting mixing furnace, and open-hearth furnaces, whose charges are partially or wholly taken from the intermediate large tilting furnace. The transfer of metal from the 50 blast furnace to the mixer and from the mixer to the open hearths may be carried out by ladles and in the usual way, or, in any other desirable manner.

In carrying out the invention, the blast 55 furnace is charged in the usual manner, except that the usual proportioning of the fur-

nace charges, particularly as to limestone and coke, is not required, since the percentage of silicon in the pig produced is immaterial. The limestone and fluxes will remove a part of the metalloids, but there is no proportioning to keep these metalloids below a definite maximum content, as now required and universally used in blast furnace practice. On account of this non-proportioning or calculating of the flux, the amount of limestone and coke may be, and preferably is, materially reduced below the amount normally used in blast furnace operations. By this manner of operating the blast furnace, I not only reduce the cost by reducing the amount of limestone and coke in the charge; but I am also enabled to increase the pig iron output of the furnace, since no attention is paid to the content of silicon and the same may be the case as to the phosphorus and sulfur. The molten pig iron thus produced, which is high in silicon, and may be relatively high in phosphorus and sulfur, is tapped preferably from a series of blast furnaces operated in this manner at successive intervals and taken to the large regenerative tilting furnace and charged therein. A constant bath of metal is maintained in this mixer, metal being successively charged into this bath from the furnaces, and successive charges of the treated metal being taken out of this mixer for the open hearths. In this mixer, the metal is mixed from the several blast furnaces, if such are employed, and by the use of the regenerators, the metal is treated to reduce the amount of silicon as well as sulfur and phosphorus. This action is carried on at a much lower temperature than that ordinarily used in open hearth treatment and may be about 1000° F. below ordinary steel making temperatures. This mixer is provided with a basic lining and the relatively low temperature prevents any appreciable attack from the silicon upon the basic lining. This preliminary treatment partially eliminates the silicon, phosphorus and sulfur, and from the mixer I tap for use in the open hearth furnaces a molten metal which is usually refined to about one-half the percentage of the silicon and a material reduction in the percentage of phosphorus and sulfur present in the standard steel making pig. Lime, or basic material or flux may be added to the mixer as required, or flux may be added in the

shape of fluid slag from the open hearth furnaces. Iron oxids also may be used to create a more rapid reaction and reduce the amount of fuel required in the mixer operation and further reduce the cost both of the metallic charge and the operation.

In tapping the partially refined metal from the mixer, the mixer is preferably tilted to discharge the proper amount into a 10 ladle and this charge is fed into one of the open hearth furnaces and preferably combined therein with low grade material which may include low grade scrap, borings of cast iron, turnings of steel, etc., high silicon pig, 15 iron oxids like scale, cinder or iron ore, or any other material containing iron. If the open hearth charge is made up partly of each class of material, the solid material is preferably charged first and brought to a 20 suitable condition and a charge of the partially refined metal from the mixer then delivered to complete the open hearth charge. The slag in the mixer is preferably not charged into the open hearth as it will be 25 considerably exhausted. In tapping the open hearth after the usual heat, which, however, may be shortened on account of the preliminary treatment in the mixer and the more violent reaction in charging molten 30 but partially refined iron or semi steel into the heated, partially melted or molten charge already in the finishing open hearth and which conditions are regulated to secure the proper degree of instantaneous reaction or 35 boiling to insure the desired or best and most economical number of heats per week; the open hearth slag may be charged back into the mixer to assist in removing or absorbing the metalloids and impurities. This slag 40 will be charged in a molten condition and will aid in protecting the basic lining from oxidation and also in protecting the furnace bottom in the mixer. These operations proceed continuously, the open hearth furnaces 45 being tapped when the heat is finished, fresh charges placed therein and made up either from a mixture of solid material with partially refined mixer metal or from the latter alone, while charges of the high silicon 50 molten pig are fed from time to time to the mixer in which the pool of partially refined metal is maintained.

The main feature of my invention therefore resides in the triplex process above described, wherein the blast furnace is run at the minimum cost for producing pig iron regardless of analysis, while the regenerative mixer partially refines this low grade pig at a relatively low cost for fuel and furnace 60 maintenance owing to the low heat or temperature required and partially removes the silicon which the slag readily absorbs even at the low temperature present. At this temperature the silicon as an acid is not so 65 active as to readily attack the basic lining,

while the slag also removes a considerable amount of phosphorous and sulfur, thus preparing the metal for the open hearth finishing furnaces in which the metal is finished into steel, either with or without partial charges of other materials, such as low grade scrap, borings, turnings, etc.

The advantages of my invention will be apparent to those skilled in the art. The process enables a blast furnace to be run with maximum economy and production giving a pig iron in which no attention is paid to the amount of silicon, sulfur and phosphorus contained. On account of the non-proportioning or calculating of the 70 charges in the usual way, the amount of limestone and coke in the blast furnace charge may be reduced and the output of pig iron increased. The time used in the open hearth heats may be considerably reduced on account of the preliminary partially refining in the tilting open hearth or mixing furnace; and low grade material, such as a poor grade of scrap and cast iron 75 borings, turnings, etc., may be worked up 80 in the open hearth furnaces in conjunction with the partially refined molten pig and steel of the finest analysis and soundness produced. Such steel may be made suitable 85 for deep stamping work, also the substantially acid proof, so called, ingot iron and similar steels, as well as the higher carbon and alloy steel used in the manufacture of 90 springs, forgings and the like. This process 95 also gives advantages in the production 100 of steel from a chromium nickel iron ore, such as certain Cuban ores. By the extra fluxing of this process the chromium can be reduced to one-half or one-third per cent, 105 this producing fine steel for rails, stampings, 110 forgings, etc., with but a fraction of the metallic loss in the direct blast furnace and Bessemer blowing followed by the basic open hearth method—in other words the duplex 115 process. A triplex system is thus afforded 120 which is of advantage both in smelting in the blast furnace and in reduction of time in the open hearth. The metalloids, such as silicon, phosphorus and sulfur are reduced and partially eliminated in the preliminary 125 mixing furnace in which the basic lining and lime conditions, if used, act for this purpose. The low temperature avoids attacking the lining in such case.

Many variations may be made in the form 120 and arrangement of the apparatus without departing from my invention.

I claim:

1. In the manufacture of steel the steps 125 consisting of smelting iron ore without reference to analysis for silicon content of the pig to produce a low grade pig, treating said pig in a basic regenerative open hearth at a temperature materially below normal steel making temperatures to partially eliminate 130

the metalloids, and then transferring the metal to and treating it in an open hearth furnace to produce steel.

2. In the manufacture of steel the steps 5 consisting in smelting iron ore in a series of blast furnaces without regard to silicon analysis, supplying molten pig from the series of blast furnaces to a regenerative open hearth furnace, maintaining a constant 10 pool therein, treating the metal therein to reduce the metalloids at a temperature materially below ordinary steel making temperatures, and transferring charges from said furnace from time to time to open hearths to 15 finish into steel.

3. In the manufacture of steel the steps consisting of smelting iron ore to produce a low grade pig without reference to metalloid analysis, and treating said pig in a regenerative open hearth furnace to partially eliminate the silicon, phosphorus and sulfur preliminary to further treatment.

4. In the manufacture of steel the steps 25 consisting of smelting the ore with limestone materially below the normal amount in blast furnace production of basic pig, partially eliminating the metalloids in a preliminary basic furnace at a temperature materially below regenerative steel making

temperatures, and charging said partially refined material into an open hearth for reduction into steel. 30

5. In the manufacture of steel the steps 35 consisting of smelting iron ore with a burden of limestone and coke materially below their normal burden in producing basic pig from similar ores, partially eliminating the metalloids in a preliminary basic furnace at a temperature materially below ordinary steel making temperatures, and transferring said 40 partially refined metal to an open hearth furnace for reduction into steel.

6. In the manufacture of steel the steps 45 consisting of mixing the molten pig metal from different sources in a basic furnace, maintaining a pool therein, treating said metal at a temperature materially below normal steel making temperatures to partially eliminate the metalloids, and transferring charges of said partially refined metal from 50 time to time to open hearth furnaces.

In testimony whereof, I have hereunto set my hand.

FRANK A. WILMOT.

Witnesses:

C. D. S. MILLER,  
R. C. WILMOT.